

# United States Patent

Falck-Muss et al.

[15] 3,649,173

[45] Mar. 14, 1972

## [54] STABILIZED AMMONIUM NITRATE

[72] Inventors: Rolf Falck-Muss, Arzew, Algeria; Daniel J. Newman, Jackson Heights, N.Y.; Sydney Atkin, Springfield, N.J.

[73] Assignee: Chemical Construction Corporation, New York, N.Y.

[22] Filed: Jan. 22, 1970

[21] Appl. No.: 5,119

[52] U.S. Cl.....23/103, 71/35

[51] Int. Cl.....C01c 1/18

[58] Field of Search.....23/103; 71/35; 252/385, 397

[56]

## References Cited

### UNITED STATES PATENTS

3,366,468 1/1968 Porter.....23/103 X  
3,317,276 5/1967 Brown, Jr. et al.....23/103

*Primary Examiner*—Oscar R. Vertiz

*Assistant Examiner*—G. O. Peters

*Attorney*—J. L. Chaboty

[57]

## ABSTRACT

Solid ammonium nitrate particles are stabilized against thermal shock and cracking at phase transition temperatures by the inclusion of small but effective amounts of silicofluoride compound, a phosphate compound and a sulfate compound in combination, within the solid ammonium nitrate particles.

9 Claims, No Drawings

## STABILIZED AMMONIUM NITRATE

## BACKGROUND OF THE INVENTION

## 1. Field of the Invention

The invention relates to the production of solid discrete particles of ammonium nitrate, and the prevention of thermal shock and cracking due to internal stress in the particles generated at phase transitions which occur due to temperature change.

## 2. Description of the Prior Art

Numerous additive compounds have been suggested, either singly or in combination, for inclusion in solid ammonium nitrate particles, in order to prevent or alleviate the well known phenomenon of thermal shock and cracking of the particles which readily occurs in pure ammonium nitrate particles when the temperature of the particles is raised or lowered through the phase transition temperatures, of which the 32°C. transition point is most significant in practice. Among those compounds which have been suggested in the prior art are phosphates such as potassium metaphosphate, mono-and di-ammonium phosphate, sulfates such as ammonium sulfate, potassium chloride, magnesium salts, calcium salts, sodium silicate, clays, nitrates such as sodium nitrate, calcium nitrate and potassium nitrate, iron cyanides, copper oxides and boron compounds. These compounds and various combinations of compounds are proposed in U.S. Pat. Nos. 1,406,455; 1,698,793; 1,868,890; 1,932,434; 1,939,165; 1,947,601; 1,966,947; 2,124,332; 2,136,069; 2,657,977; 2,702,747; 2,879,133; 2,901,317; 2,943,928; 2,957,763; 3,007,773; 3,018,164; 3,021,207; 3,026,193; 3,030,179; 3,034,853; 3,034,858; 3,070,435; 3,116,108; 3,117,835; 3,148,945 and 3,317,276. The inhibition of calcium nitrate formation in the production of nitrochalk by silicofluoride addition is disclosed in U.S. Pat. No. 3,351,454.

## SUMMARY OF THE INVENTION

In the present invention, it has been determined that an improved solid ammonium nitrate composition may be produced in the form of discrete particles which resist thermal shock and cracking due to deformation at phase transition temperatures such as 32°C., by the inclusion of a synergistic combination of compounds into the solid ammonium nitrate, preferably by the addition of small but effective amounts of these compounds to molten ammonium nitrate prior to solidification of the ammonium nitrate as discrete particles by prilling or the like. The molten ammonium nitrate is preferably initially in the form of a substantially anhydrous melt, however in some cases the melt may contain water in an amount up to about 5 percent by weight. The additive compounds employed in combination in the present invention are a silicofluoride compound, a phosphate compound and a sulfate compound. Numerous compounds within each of these categories may be effectively employed to stabilize ammonium nitrate. Among the feasible silicofluoride compounds are ammonium silicofluoride, sodium silicofluoride, potassium silicofluoride, magnesium silicofluoride and zinc silicofluoride, or mixtures of these compounds. Usable phosphate compounds include monoammonium phosphate, diammonium phosphate, trisodium phosphate and mixed fertilizer compositions which include phosphatic fertilizer components. Among the many sulfate compounds which may be employed in the present invention are ammonium sulfate, sodium sulfate, potassium sulfate and calcium sulfate. A preferred method of adding a phosphate compound and a sulfate compound to the molten ammonium nitrate is by the addition of phosphoric acid and sulfuric acid to the molten ammonium nitrate, or to its precursor nitric acid, followed by in situ neutralization of the acids by addition of a suitable base or basic solution to the molten ammonium nitrate. Typical feasible basic materials for this purpose include ammonia, sodium hydroxide, sodium carbonate, potassium hydroxide and potassium carbonate, and these bases may be added either in the anhydrous state or as aqueous solutions. The molten ammonium nitrate containing

the additive compounds of the present invention in combination is preferably solidified in the form of discrete particles by a prilling procedure, in which the molten ammonium nitrate is sprayed into an airstream, so that the resulting ammonium nitrate droplets solidify in the airstream in the form of spherical solid prills. The resultant prills preferably contain up to about 0.5 percent by weight of each of the additive compounds, and in accordance with the present invention the resulting prills are highly resistant to thermal shock and cracking at the phase transition temperatures such as 32°C. Alternative methods of solidifying the molten ammonium nitrate in the form of discrete particles after additives addition include granulation, crystallization, or by flowing the molten ammonium nitrate onto a chilled belt on which the molten material solidifies in the form of a thin sheet or film which is then broken up into small crystals or particles.

The principal advantage of the present invention is that the resulting solid ammonium nitrate composition is stabilized against thermal shock and cracking at phase transition temperatures, so that the product may be safely stored for extended periods of time without the development of a dusting or caking problem. Another advantage is that the production of fines or powdered material during the preparation of the discrete solid particles by prilling or the like is substantially reduced, so that the recycle of fines is reduced in the ammonium nitrate production facility, which reduces the capital and operating costs such as by decreasing stream consumption for concentration of remelt solutions. A further advantage is that the additive compounds of the present invention are relatively inexpensive, and in most cases these additives are readily available at fertilizer complexes or production sites, especially when phosphatic fertilizers are concomitantly produced from phosphate rock, phosphatic shales or the like. Silicofluorides are generally produced and recovered as byproducts in the processing of phosphatic raw materials to produce phosphate products, as for example in the production of phosphoric acid as described in U.S. Pat. No. 2,905,535. An additional advantage is that the additive compounds of the present invention can be disseminated and dissolved into the molten ammonium nitrate, and the provision of special or ancillary mixing equipment or apparatus is minimized.

It is an object of the present invention to provide an improved solid ammonium nitrate product.

Another object is to prevent thermal shock and cracking of solid ammonium nitrate particles at phase transition temperatures, by the addition of a synergistic combination of additive compounds to the ammonium nitrate.

A further object is to produce improved ammonium nitrate prills which are resistant to thermal shock and cracking at phase transition temperatures, and which may be safely stored for extended periods of time without dusting or caking.

An additional object is to reduce the amount of fines and powder which are formed when molten ammonium nitrate is converted to discrete solid particles by prilling or the like.

An object is to provide an improved method of stabilizing solid ammonium nitrate particles against thermal shock and cracking at phase transition temperatures, by employing a combination of additive compounds in the ammonium nitrate including a silicofluoride compound, a phosphate compound and a sulfate compound.

These and other objects and advantages of the present invention will become evident from the description which follows.

## DESCRIPTION OF PREFERRED EMBODIMENTS

Ammonium nitrate crystals or prills without additives undergo volume expansion and contraction as they pass through the phase transition temperatures such as 32° and 83°C., causing the prills to break down into fine particles or dust. The effect of various additives including the additives combination of the present invention was investigated on a laboratory scale, followed by further testing in a commercial facility,

which demonstrated the improved results obtained by the present invention.

In all cases, the prills were subjected to a number of temperature changes through a range which included a phase transition temperature, and the percentage of prills cracked from thermal shock at various numbers of transition was determined. Following are the results obtained in the laboratory scale and commercial plant facility tests.

#### EXAMPLE I. — LABORATORY SCALE TESTS

The ammonium nitrate prills produced in the laboratory were obtained by spraying a melt consisting of 99.5 percent ammonium nitrate plus additive from a gun containing 0.029 inch holes using about 10 p.s.i.g. nitrogen pressure. In order to obtain more failing height, the spray was arched from the top of a 27-feet-high platform toward the ceiling and allowed to fall to the floor. The prills produced in this manner contained considerable irregularly shaped prills and were weaker than prills produced in a commercial plant, but otherwise had characteristics similar to commercial prills.

TABLE I.

#### TYPICAL SCREEN ANALYSIS OF LABORATORY PRILLS

| Mesh Size   | % By Weight |
|-------------|-------------|
| +6 mesh     | 0.0         |
| -6+8 mesh   | 9.1         |
| -8+10 mesh  | 33.3        |
| -10+14 mesh | 43.3        |
| -14 mesh    | 14.3        |

For the phase transition tests, only -8 + 10 mesh prills were used. Two different series of test were made to determine the resistance of ammonium nitrate prills produced without and with various additives, to thermal shock and cracking due to repeated passage through transition temperatures. In the first series of tests, prills were heated in an oven at 42°C. for 2 hours and then allowed to cool to room temperature at 23°C. for 2 hours. The temperature changes thus provided for a transit of the phase transition temperature of 32°C. After each cycle, the percentage of unbroken prills was recorded. In the second series of tests, the prills were cycled between 91° and 42°C. at 2 hour intervals, to provide for a transit of the phase transition temperature of 83°C. Following is data relative to the inclusion of additives in the prills.

TABLE II

#### ADDITIVE INCLUSION IN PRILLS

| Run Nos.  | Additive (S) Added      | % By Weight |
|-----------|-------------------------|-------------|
| 1 and 14  | none                    | 0           |
| 2 and 15  | ammonium sulfate        | 0.2         |
| 2 and 15  | diammonium phosphate    | 0.2         |
| 2 and 15  | sodium silicofluoride   | 0.2         |
| 3 and 16  | diammonium phosphate    | 0.6         |
| 4 and 17  | ammonium sulfate        | 0.6         |
| 5 and 18  | ammonium sulfate        | 0.3         |
| 5 and 18  | diammonium phosphate    | 0.3         |
| 6 and 19  | sodium silicofluoride   | 0.6         |
| 7 and 20  | ammonium silicofluoride | 0.6         |
| 8 and 21  | potassium metaphosphate | 0.6         |
| 9 and 22  | potassium metaphosphate | 0.3         |
| 9 and 22  | sodium silicofluoride   | 0.3         |
| 10 and 23 | boric acid              | 0.6         |
| 11 and 24 | boric acid              | 0.3         |
| 11 and 24 | sodium silicofluoride   | 0.3         |
| 12 and 25 | aluminum phosphate      | 0.6         |
| 13 and 26 | calcium carbonate       | 0.3         |
| 13 and 26 | ammonium sulfate        | 0.3         |

TABLE III.—EFFECT OF ADDITIVES ON PRILL BREAKAGE FROM THERMAL SHOCK AT 32° C. PHASE TRANSITION

| Run No.: | Number of transitions                                           |    |    |     |       |       |       |
|----------|-----------------------------------------------------------------|----|----|-----|-------|-------|-------|
|          | 3                                                               | 5  | 8  | 11  | 14    | 17    | 20    |
|          | Percent prills cracked from thermal shock (42° C.-23° C. cycle) |    |    |     |       |       |       |
| 1        | 32                                                              | 48 | 80 | 84  | 96    | 100   | ----- |
| 2        | 0                                                               | 0  | 0  | 4   | 62    | 100   | ----- |
| 3        | 24                                                              | 32 | 48 | 80  | 92    | 100   | ----- |
| 4        | 4                                                               | 12 | 20 | 24  | 28    | 44    | 64    |
| 5        | 0                                                               | 4  | 28 | 40  | 80    | 100   | ----- |
| 6        | 36                                                              | 68 | 76 | 88  | 92    | 96    | 100   |
| 7        | 32                                                              | 40 | 40 | 56  | 60    | 72    | 88    |
| 8        | 0                                                               | 16 | 28 | 60  | 100   | ----- | ----- |
| 9        | 12                                                              | 28 | 72 | 100 | ----- | ----- | ----- |
| 10       | 16                                                              | 28 | 32 | 40  | 76    | 76    | 88    |
| 11       | 4                                                               | 4  | 4  | 4   | 4     | 16    | 16    |
| 12       | 0                                                               | 4  | 8  | 12  | 36    | 60    | 100   |
| 13       | 4                                                               | 28 | 28 | 52  | 82    | 100   | ----- |

From the results in Table III, it is evident that the combination of additives of the present invention, as provided in Run No. 2, attained the greatest improvement up to 11 transitions of all of the additives or additive combinations tested, as compared to Run No. 1 in which no additive was present in the ammonium nitrate.

TABLE IV.—EFFECT OF ADDITIVES ON PRILL BREAKAGE FROM THERMAL SHOCK AT 83° C. PHASE TRANSITION

| Run No.: | Number of transitions                                           |    |    |    |    |    |    |
|----------|-----------------------------------------------------------------|----|----|----|----|----|----|
|          | 3                                                               | 5  | 8  | 11 | 14 | 17 | 20 |
|          | Percent prills cracked from thermal shock (91° C.-42° C. cycle) |    |    |    |    |    |    |
| 14       | 8                                                               | 32 | 40 | 48 | 48 | 60 | 68 |
| 15       | 0                                                               | 0  | 0  | 0  | 0  | 0  | 0  |
| 16       | 4                                                               | 4  | 4  | 8  | 12 | 28 | 32 |
| 17       | 0                                                               | 0  | 0  | 0  | 4  | 4  | 8  |
| 18       | 0                                                               | 0  | 4  | 4  | 12 | 12 | 12 |
| 19       | 12                                                              | 12 | 32 | 40 | 44 | 60 | 64 |
| 20       | 12                                                              | 20 | 48 | 52 | 60 | 64 | 68 |
| 21       | 0                                                               | 0  | 0  | 0  | 4  | 4  | 4  |
| 22       | 0                                                               | 0  | 0  | 8  | 12 | 16 | 16 |
| 23       | 0                                                               | 0  | 8  | 12 | 12 | 16 | 20 |
| 24       | 0                                                               | 0  | 0  | 0  | 0  | 0  | 8  |
| 25       | 0                                                               | 0  | 0  | 0  | 4  | 4  | 4  |
| 26       | 0                                                               | 0  | 4  | 8  | 12 | 12 | 20 |

From the results in Table IV, it is evident that the combination of additives of the present invention, as provided in Run No. 15, provided complete stabilization of the ammonium nitrate and attained the greatest improvement of all of the additives or additive combinations tested, as compared to Run No. 14 in which no additive was present in the ammonium nitrate.

#### EXAMPLE II. — COMMERCIAL PLANT TESTS

Test were conducted at a commercial ammonium nitrate production facility to confirm the laboratory results of Example I. The facility was operated at a production rate of 300 tons/day of prilled ammonium nitrate. Initial prilled ammonium nitrate samples were taken without the addition of stabilizer, and further samples were taken after the stabilizer of the present invention was added to the molten ammonium nitrate prior to prilling the melt. Samples were taken at the prill cooler outlet, which discharged prills without stabilizer addition at a temperature of 50°C. With the addition of stabilizer, prill cooler exit temperature was reduced to 38° or 29°C. as indicated infra. The stabilizer was an aqueous solution made at the site and consisting (by weight) of 75.4 percent water and 8.2 percent each of sodium silicofluoride, ammonium sulfate and 18-46-0 fertilizer, the latter component consisting principally of diammonium phosphate. The fertilizer was dissolved in water, decanted and screened to remove sand and other insolubles. The stabilizer was constantly agitated and held at 66°C. by steam coils.

After taking dry run samples without additive addition, the

stabilizer feed pump was set at 1 gallon/minute and addition of additive was initiated. The outlet temperature of the cooler was reduced. After running for about 1 hour with stabilizer addition, it was observed that the prills on the conveyor appeared larger, and the screen reject flow had diminished considerably. Screen reject remained at a low figure throughout the balance of the stabilizer addition test. Following are the test results obtained, relative to the effect of the additive on prill breakage from thermal shock at the 32°C. transition point.

TABLE V

## ADDITIVE INCLUSION IN PRILLS (BY ANALYSIS)

| Run No. | Percent By Weight<br>Diammonium<br>Phosphate | Percent By Weight<br>Ammonium<br>Sulfate | Percent By Weight<br>of Additive<br>Sodium<br>Silicofluoride |
|---------|----------------------------------------------|------------------------------------------|--------------------------------------------------------------|
| 1       | 0                                            | 0                                        | 0                                                            |
| 2       | 0.10                                         | 0.08                                     | 0.12                                                         |
| 3       | 0.095                                        | 0.08                                     | 0.13                                                         |

TABLE VI

## PLANT OPERATING CONDITION

| Run No. | Prill Cooler<br>Exit Temperature |
|---------|----------------------------------|
| 1       | 50°C.                            |
| 2       | 38°C.                            |
| 3       | 29°C.                            |

TABLE VII.—EFFECT OF STABILIZER ON PRILL BREAKAGE FROM THERMAL SHOCK AT 32° C. PHASE TRANSITION

| Run No.:                                                           | Number of transitions |   |    |    |    |    |    |
|--------------------------------------------------------------------|-----------------------|---|----|----|----|----|----|
|                                                                    | 3                     | 6 | 9  | 12 | 15 | 18 | 21 |
| Percent prills cracked from thermal shock<br>(42° C.-23° C. cycle) |                       |   |    |    |    |    |    |
| 1.....                                                             | 0                     | 8 | 20 | 20 | 24 | 24 | 28 |
| 2.....                                                             | 0                     | 0 | 0  | 0  | 0  | 0  | 4  |
| 3.....                                                             | 0                     | 0 | 0  | 4  | 4  | 4  | 8  |

The greatly improved results obtained in Run Nos. 2 and 3 due to stabilizer addition, as compared to Run No. 1 in which no stabilizer additives were provided, clearly indicate the commercial advantages of the invention in stabilizing am-

monium nitrate against thermal shock at phase transitions. It should be noted that without the additive, prills cannot be cooled below 50°C. without greatly excessive breakage.

We claim:

- 5 1. A method of stabilizing solid ammonium nitrate particles against thermal shock at phase transition temperatures which comprises adding a small but effective amount of a silicofluoride compound, a phosphate compound and a sulfate compound to molten ammonium nitrate, whereby said compounds are distributed in said molten ammonium nitrate, and solidifying said molten ammonium nitrate in the form of discrete particles, said solid ammonium nitrate particles containing said compounds in sufficient proportion to render said particles resistant to cracking from thermal shock at phase transition temperatures.
- 10 2. The method of claim 1, in which said molten ammonium nitrate contains water in an amount up to about 5 percent by weight.
- 15 3. The method of claim 1, in which said silicofluoride compound is selected from the group consisting of ammonium silicofluoride, sodium silicofluoride, potassium silicofluoride, magnesium silicofluoride and zinc silicofluoride.
- 20 4. The method of claim 1, in which said phosphate compound is selected from the group consisting of monoammonium phosphate, diammonium phosphate and trisodium phosphate.
- 25 5. The method of claim 1, in which said sulfate compound is selected from the group consisting of ammonium sulfate, sodium sulfate, potassium sulfate and calcium sulfate.
- 30 6. The method of claim 1, in which said phosphate compound and said sulfate compound are added to said molten ammonium nitrate by adding phosphoric acid and sulfuric acid to said molten ammonium nitrate during production of the ammonium nitrate, and neutralizing said acids within said molten ammonium nitrate by the addition of a base selected from the group consisting of ammonia, sodium hydroxide, sodium carbonate, potassium hydroxide and potassium carbonate.
- 35 7. The method of claim 1, in which said molten ammonium nitrate containing said compounds is solidified in the form of discrete particles by spraying said molten ammonium nitrate into an air stream, whereby said molten ammonium nitrate flows downwards through said air stream as discrete droplets which solidify in the form of prills.
- 40 8. The method of claim 1, in which each of said compounds is added to said molten ammonium nitrate in a proportion up to about 0.5 percent by weight of said molten ammonium nitrate.
- 45 9. A solid ammonium nitrate composition stabilized against thermal shock at phase transition temperatures which comprises ammonium nitrate containing small but effective amounts of a silicofluoride compound, a phosphate compound and a sulfate compound.

UNITED STATES PATENT OFFICE  
CERTIFICATE OF CORRECTION

Patent No. 3649173 Dated March 14, 1972

Inventor(s) R. Falck-Muus, D. J. Newman, S. Atkin

It is certified that error appears in the above-identified patent and that said Letters Patent are hereby corrected as shown below:

Col. 2 line 28, read "steam" instead of "stream". Also line 71, read "32°C" instead of "32°".

Col. 3 line 6, read "transitions" instead of "transition". Also line 46, read "91°C" instead of "91°". Also line 47, read "intervals" instead of "internals".

Claim 1 line 3 (col. 6 line 7) after "adding", delete "a" and read "the combination of". Also read "amounts" instead of "amount". Also read "at least about 0.12% by weight of" after "of".

Claim 9 line 4 (col. 6 line 52) read "at least about 0.12% by weight of" after "of".

Signed and sealed this 29th day of August 1972.

(SEAL)

Attest:

EDWARD M. FLETCHER, JR.  
Attesting Officer

ROBERT GOTTSCHALK  
Commissioner of Patents